

Jan. 25, 1927.

1,615,387

H. W. JESPERSEN

METHOD OF AND APPARATUS FOR COATING CORES

Filed March 23, 1923



Fig. 3.



Fig. 4.



Fig. 5.



Fig. 6.



Fig. 7.



Inventor  
Helgo W. Jespersen  
by *H.G. Patterson*.

Atty.

## UNITED STATES PATENT OFFICE.

HELGO WIGGO JESPERSEN, OF RIVERSIDE, ILLINOIS, ASSIGNOR TO WESTERN ELECTRIC COMPANY, INCORPORATED, OF NEW YORK, N. Y., A CORPORATION OF NEW YORK.

## METHOD OF AND APPARATUS FOR COATING CORES.

Application filed March 23, 1923. Serial No. 627,202.

This invention relates to a method of and apparatus for coating cores.

An object of the invention is to produce a core having a coating of pulp thereon which is attached to the core solely by intermingling of the fibers thereof and without the use of any adhesive substance.

Another object of the invention is to coat a plurality of cores in strand form simultaneously.

Briefly, the method consists in engaging a core with a screen or other suitable foraminous member, depositing pulpos material on the core and the foraminous member, removing the core and the pulpos material in ribbon form from the foraminous member, reducing the width of the ribbon, and then forming the ribbon on the core to constitute a homogeneous coating therefor. When a plurality of cores are coated simultaneously the method consists in bringing these cores simultaneously into engagement with the foraminous member, depositing pulpos material upon the foraminous member and the plurality of cores in contact therewith, removing the cores and the sheet of pulpos material supported thereby from the foraminous member, slitting the sheet into a plurality of ribbons individual to the cores, and then forming the ribbons on the cores to constitute a homogeneous coating therefor.

The present method may be employed to advantage for insulating electrical conductors, but it is to be understood that it is not limited to this purpose but only in so far as is defined by the appended claims. Where the method is used in insulating electrical conductors, manila, wood, rag, cotton, esparto, jute, hemp, and asbestos pulps may be employed as the coating material, but other materials than those specified may be used without departing from the spirit and scope of the present invention which contemplates in its broadest aspect the coating of any core with pulp of any material.

The drawings illustrate an apparatus by which the method may be practiced, the apparatus being especially designed for coating cores in strand form, but it is to be understood that other apparatus may be devised for coating cores in other forms without departing from the spirit and scope of the invention.

The word "pulp" as used in the specifica-

tion and claims is to be understood as defining and including any cohering fibrous mass whether suspended in a liquid, moist or substantially dry.

In the accompanying drawings,

Fig. 1 is a side elevation of a preferred apparatus by which the method may be practiced;

Fig. 2 is an enlarged fragmentary top plan view of a portion of the apparatus shown in Fig. 1;

Figs. 3, 4 and 5 are enlarged sectional views showing the form of the pulp coatings at they leave the felt associated with the foraminous member, as they are being acted upon by the slitting mechanism, and as they are delivered from the squeeze rolls respectively; and

Figs. 6 and 7 are enlarged sectional views showing the form of the pulp coatings during the forming operation and after the completion of such operation respectively.

The steps of the method may be readily understood from a detailed description of the apparatus by which the method may be practiced.

Referring to the drawings in detail in which like reference numerals designate similar parts throughout the several views, the apparatus comprises a drum 10 whch is partially submerged in a liquid containing pulp within a trough 11. The drum 10 comprises a pair of metal sides and a peripheral portion 12 secured thereto. The portion 12 is provided with a plurality of relatively large perforations 13 which are covered with a strip of fine wire mesh 14 as shown in Fig. 2. The drum has a centrally disposed tubular axle 15 which is rotatably mounted in suitable bearings 16 carried by a framework 17 which supports all of the elements of the apparatus.

Pulpos material is strained onto the wire mesh 14 as the drum 10 is rotated in the tank by maintaining the level of the mixture within the drum 10 at a lower level than that of the pulp liquid in the tank 11 as indicated by dotted lines A and B respectively. This difference in levels is maintained by a siphon pipe 18 which has its inlet opening submerged in the liquid of the drum and its discharge through the tubular axle 15. The continuous circulation of the pulp liquid is maintained in the tank 11 by feeding the

pulp liquid from a supply tank (not shown) into the tank 11 by means of a pipe 19, and out of said tank through a pipe 20 into a receiving tank (not shown) from which it 5 is pumped back into the supply tank in any suitable manner. As the drum 10 rotates in the tank 11, due to the difference in levels of the liquid in the drum and the tank, the liquid in the tank will pass through the wire 10 mesh 14 and perforations 13, straining the pulp carried by such liquid onto the outer surface of the wire mesh.

Disposed in contact with the wire mesh 14 is a roll 21, preferably covered with felt 15 and mounted upon a pair of brackets 24. The cores to be coated are fed from suitable supply spools 30 over idler rolls 31 and into contact with the pulpy material which has been deposited on the foraminous screen 14, 20 and as the drum 10 is rotated the cores are carried into the liquid containing pulpy material, and when the pulpy material is deposited upon the foraminous member it also covers the cores in engagement therewith. The idler rolls 31 are spaced from the periphery 12 of the drum 10 so that the cores are held out of contact with that section of the foraminous member which is near the surface of the liquid in the tank whereby 25 pulp is strained onto such section before the strands or cores are brought into contact therewith. The first deposit of pulp on the foraminous member is indicated by the letter C, while as the drum rotates in the tank, 30 additional amounts of pulpy material will be deposited on the core and the associated foraminous member, forming a thicker coating indicated by the letter D. The drum 10 is rotated in the direction indicated by the 35 arrow and the pulp on the foraminous covering together with the associated cores are brought into contact with a felt covered roll 24. The periphery of this roll has a foraminous portion formed of fine wire mesh and 40 when the pulp on the foraminous portion of the drum is brought into contact therewith, the "free liquid" so to speak in the pulp mixture will be squeezed out, partially through the foraminous portion of the drum 45 0 10 and partially through the felt and the associated foraminous portion of roll 24. The partially dried pulp adheres to the felt in a sheet form with the cores included therein. 50 The cores then pass partially around the felt covered roll 21, which serves to remove the deposited material from the foraminous member, and a roll 23 provided with suitable tension means to press it against the 55 0 10 felt roll 21, serves to attach the sheet of pulpy material to the cores to some extent as shown in Fig. 3. When the sheet supported by the cores is subjected to the action of a cutter 28 bearing upon the periphery of 60 0 15 a drum 26, the sheet is slit into two ribbons.

Each core and its associated ribbon tends to remain in close contact, the cores being disposed substantially in the center of the ribbons as shown in Fig. 4. From the slitting disc 28 the two ribbons and their associated cores are passed between pairs of squeeze rolls 40 and 41. These squeeze rolls serve to remove additional moisture from the pulpy ribbons and force the fibers thereof into more intimate contact as shown in Fig. 75 5. From the squeeze rolls 40 and 41 the cores and the associated ribbons are drawn through forming mechanisms 33 and 34 which are associated with the pairs of squeeze rolls 40 and 41 respectively. 80

The formers 33 and 34 wrap the projecting edges of the ribbons around the cores and around each other, the appearance of the coating as they are first acted upon by the formers and after forming action is completed being clearly shown in Figs. 6 and 7 respectively. Each of the formers causes a thorough intermingling of the pulp fibers of the ribbon and shapes the coating so that it embraces the core and conforms to the 90 shape thereof. Furthermore, the coating is molded into a mass so homogeneous that upon cutting the core and the associated coating, the latter will not fray or ravel and will not become easily detached from the 95 core.

Each of the formers 33 and 34 comprises essentially two plates which are rotated around the core and serve to wrap the associated pulp ribbon therearound in much the same manner as though the core and pulp ribbon were rolled on a table top with the palm of the hand. The formers 33 and 34 shown in the drawings are identical with that fully described in the co-pending application of Walker and March, Serial No. 547,923, filed March 29, 1922, and for a detailed description of this mechanism reference is made to the application above referred to. 100

Each of the coated cores is drawn from its associated former and subjected to a mechanism for thoroughly drying out the coating. The means for performing this operation comprises pairs of wide hollow drums 35 and 36 internally heated and having a plurality of grooves (not shown) formed on the periphery thereof which receive the coated cores, guides (not shown) being provided for directing the core over first one drum of each pair and then over the other drum until it has traversed all of the grooves on both drums, after which the cores are stored on take-up spools 37 and 38 respectively. The drying apparatus shown is identical with that fully illustrated and shown in the Walker-March co-pending application above referred to and reference is made to the said application for a full disclosure of this 110 115 120 125 130 135 apparatus.

The apparatus illustrated and above described is adapted to simultaneously coat two cores in strand form, but it is to be understood that the machine can be modified

5 and the parts duplicated to simultaneously coat a larger number of cores without departing from the spirit and scope of the present invention.

Although it has been stated that the primary object of the invention is to apply a 10 coating of pulp to a core without the use of any adhesive substance, the machine herein disclosed may be used with a pulp mixture containing a sizing substance, or the pulp 15 may be deposited on a core which has been previously treated with an adhesive agent without departing from the spirit and scope of the present invention.

What is claimed is:

20 1. The method of coating a core in strand form with pulp, which consists in associating a core with a foraminous member, depositing pulpous material in liquid suspension upon the member and the core, removing the core and the material from the member, removing some of the material from the core, and then forming the remaining portion of the said material on the core to constitute a coating therefor conforming 25 with the shape of the core and held on the core by an intermingling of the pulp fibers.

20 2. The method of coating a core in strand form with pulp, which consists in associating a core with a foraminous member, depositing pulpous material in liquid suspension upon the member and the core, removing the core and the deposited material from the member in ribbon form, reducing the width of the ribbon, and then forming the 30 ribbon on the core to constitute a coating therefor conforming with the shape of the core and held on the core by an intermingling of the pulp fibers.

35 3. The method of coating a core in strand form with pulp, which consists in associating a core with a foraminous member, depositing pulpous material in liquid suspension upon the foraminous member and upon the core, removing the core and the deposited material from the member and removing some of the moisture therefrom, removing some of the material, and then forming the remaining material on the core to constitute a coating therefor conforming with the 40 shape of the core and held on the core by an intermingling of the pulp fibers.

45 4. The method of coating a core in strand form with pulp, which consists in associating a core with a foraminous member, depositing pulpous material in liquid suspension upon the foraminous member and the core, removing the core and the material from the member and removing some of the moisture therefrom to form a ribbon there- 50 of, reducing the width of the ribbon, and

then forming the ribbon on the core to constitute a coating therefor conforming with the shape of the core and held on the core by an intermingling of the pulp fibers.

5. The method of coating a core in strand form with pulp, which consists in associating a core with a foraminous member, depositing pulpous material in liquid suspension upon the member and the core, removing the core and the material from the member and removing some of the moisture therefrom, removing some of the material from the core, forming the remaining material on the core to constitute a coating therefor conforming with the shape of the core and held on the core by an intermingling of the pulp fibers, and then removing substantially all of the moisture from said coating.

6. The method of simultaneously coating a plurality of cores in strand form with pulp, which consists in associating the cores with a foraminous member, depositing pulpous material in liquid suspension upon the member and upon the cores, removing the cores and the deposited material supported thereby in sheet form from the foraminous member, separating the material into portions sufficient for each core, and forming the separated portions on the cores to constitute coatings therefor conforming with the shape of the core and held on the core by an intermingling of the pulp fibers.

7. The method of simultaneously coating a plurality of cores in strand form with pulp, which consists in associating a plurality of cores with a foraminous member, depositing pulpous material in liquid suspension upon the cores and upon the member, removing the cores and the deposited material from the foraminous member, separating the sheet of deposited material carried by the cores into ribbons individually associated with the cores, and then forming said ribbons on the cores to constitute coatings therefor conforming with the shape of the core and held on the core by an intermingling of the pulp fibers.

8. The method of simultaneously coating a plurality of cores in strand form with pulp, which consists in associating a plurality of cores with a foraminous member, depositing pulpous material in liquid suspension upon the member and upon the cores, removing the cores and the material from the foraminous member and removing a portion of the moisture from the material to form a sheet supported by the cores, separating the sheet into ribbons individual to the cores, and forming the ribbons on the cores to constitute coatings therefor conforming with the shape of the core and held on the core by an intermingling of the pulp fibers.

9. The method of simultaneously coating

a plurality of cores in strand form with pulp, which consists in associating a plurality of cores with a foraminous member, depositing pulpous material in liquid suspension upon the foraminous member and upon the cores, removing the cores and the deposited material from the foraminous member and removing some of the moisture from the material to constitute a sheet supported by the cores, separating the sheet into ribbons individual to the cores, removing additional moisture from the ribbons, forming the ribbons around the cores to constitute coatings therefor conforming with the shape of the core and held on the core by an intermingling of the pulp fibers, and removing substantially all of the remaining moisture from the cores.

10. A method of coating a core in strand form with pulp, which consists in making a ribbon of pulpous material, causing a core to engage the ribbon, applying additional pulpous material to the core and ribbon, removing a portion of the pulpous material carried by the core, and forming the remaining material into a coating for the core conforming with the shape thereof.

11. In a machine for simultaneously coating a plurality of cores in strand form, a member, means for associating the cores with the member, a receptacle containing a supply of liquid containing pulp, means for causing relative movement between the member and the liquid whereby pulp is deposited on the member and on the cores, means for removing the cores and the deposited pulp from the member in sheet form, means for cutting the sheet into ribbons individual to the cores, and means for forming the ribbons on the cores to constitute coatings therefor conforming with the shape of the core and held on the core by an intermingling of the pulp fibers.

12. In a machine for simultaneously coating a plurality of cores in strand form with pulp, a member, means for associating the plurality of cores with the member, a receptacle containing a supply of liquid containing pulp, means for causing relative movement between the member and the liquid whereby pulp is deposited upon the member

and upon the cores, means for simultaneously removing the cores and associated pulp in sheet form from the member and for removing some of the moisture from the sheet, means for cutting the sheet into ribbons individual to the cores, and means for forming the ribbons on the cores to constitute coatings therefor conforming with the shape of the core and held on the core by an intermingling of the pulp fibers.

13. In a machine for simultaneously coating a plurality of cores in strand form with pulp, a member, means for associating the cores with the member, a receptacle containing a supply of liquid containing pulp, means for causing relative movement between the member and the liquid whereby pulp is deposited upon the member and upon the cores, means for removing the cores and the associated pulp in sheet form from the foraminous member, means for separating the sheet into ribbons individual to the cores, means for removing moisture from the ribbons, and means for forming the ribbons on the cores to constitute coatings therefor conforming with the shape of the core and held on the core by an intermingling of the pulp fibers.

14. In a machine for simultaneously coating a plurality of cores in strand form with pulp, a member, means for associating the cores therewith, a receptacle containing a supply of liquid containing pulp, means for causing relative movement between the member and the liquid whereby pulp is deposited upon the member, means for simultaneously removing the cores and the deposited material from the member and for removing moisture from the material, means for cutting the material into ribbons individual to the cores, means for removing moisture from the ribbons, means for forming the ribbons on the cores to constitute coatings therefor conforming with the shape of the core and held on the core by an intermingling of the pulp fibers, and means for removing substantially all of the remaining moisture from the coatings.

In witness whereof, I hereunto subscribe my name this 9th day of March, A. D. 1923.

HELGO WIGGO JESPERSEN.